

**1**

3,824,116

**STENCIL SHEET AND METHOD OF MAKING AN  
IMAGED STENCIL SHEET**

Bror E. Anderson, Arlington Heights, and Margery L. Schick, Mount Prospect, Ill., assignors to Weber Marking Systems, Inc., Arlington Heights, Ill.

No Drawing. Continuation-in-part of application Ser. No. 27,135, Apr. 9, 1970, now Patent No. 3,704,155. This application May 15, 1972, Ser. No. 253,358

Int. Cl. B41m 1/24

U.S. Cl. 117—35.5

17 Claims

**ABSTRACT OF THE DISCLOSURE**

A stencil sheet of the type including an ink-impervious coating of a heat-flowable composition of thermoplastic film-forming material comprising a cellulose organic ester, and plasticizing material partially but incompletely compatible with the film-forming material, incorporates a polymeric hydrocarbon resin in the coating thereof for minimizing oil transfer from the stencil. The stencil sheet may be imaged thermographically and also mechanically in preferred embodiments.

**RELATED APPLICATION**

This is a continuation-in-part of application Ser. No. 27,135, filed Apr. 9, 1970, now U.S. Pat. No. 3,704,155.

**BACKGROUND OF THE INVENTION**

This invention relates to a stencil sheet of the type which includes a layer of a heat-flowable composition and to a method of making an imaged stencil sheet therewith by subjecting image areas of the stencil sheet to heat generated by infrared ray absorption.

U.S. Pat. No. 3,694,245, granted Sept. 26, 1972, on application Ser. No. 136,373, filed Apr. 22, 1971, by the present inventors as a continuation-in-part of Ser. No. 674,153, filed Oct. 10, 1967 and now abandoned, discloses a thermographic stencil sheet including an ink-pervious base sheet and an ink-impervious coating thereon of a heat-flowable composition of cellulose organic ester film-forming material and plasticizing material partially but incompletely compatible with the film-forming material. The stencil sheet is now in widespread commercial use. It is employed preferably in a stencil sheet assembly including a contacting absorbent sheet on one surface thereof, and a more rigid backing sheet on the opposite surface thereof and to which the absorbent sheet and the stencil sheet are mounted. In use, an original, such as a typed or printed sheet, is inserted between the stencil sheet and the backing sheet, and the assembly is exposed to infrared radiation on the face side of the absorbent sheet in a thermal copier such as a Weber Thermal Imager (Weber Marking Systems) or a Thermo-Fax machine (3M Company). Heat is generated in the radiation absorptive graphic portions of the original to cause the stencil sheet composition to flow in corresponding areas and thereby produce corresponding image openings in the stencil sheet. A portion of the composition rendered flowable is absorbed by the absorbent sheet and/or adjoining areas of the stencil sheet. The original and the absorbent sheet are separated from the imaged stencil sheet, the stencil sheet and the backing sheet are placed on a mimeograph duplicating machine followed by separation of the backing sheet, and the machine is operated to produce multiple mimeograph copies of the original.

It was found in use that "oil" was transferred from the stencil sheet to the original in the image areas. The oil frequently broadened and feathered the copy on the typed original (smudging), and the presence of oil on the original was not a desirable condition. The smudging

**2**

of the original affected the imaging speed in subsequent exposures, owing to the broadening of the image characters or transfer from the original to the stencil sheet. Subsequent performance was affected when the original was removed from the file for rerun, or in the event that optimum exposure was not used in imaging the first stencil.

It would be desirable to reduce the oil transfer to more desirable limits while preserving the advantageous properties of the stencil sheet of our aforesaid application.

10 In copending U.S. Pat. application Ser. No. 27,135, filed Apr. 9, 1970 by the present inventors, an improved thermographic stencil sheet exhibiting low oil transfer is claimed. The stencil sheet includes a heat-flowable composition that forms a cooled melt having a limited pourable liquid volume, and plasticizing material in the composition having limited tack and aniline point.

The improved stencil sheet claimed in the latter copending application has markedly improved oil transfer properties and in many cases also provides improved copy quality. Nevertheless, there remains room for improvement. Thus, various embodiments of the latter application do not exhibit optimum results for all of the more significant stencil performance characteristics, including imaging speed, imaging quality, oil smudging and oil transfer, and durability. Frequently, blocking occurs when oiling is reduced to a minimum. In some cases, oiling can not be reduced to the preferred low level. At times, imaging speed or imaging quality is less than optimum.

It would be desirable to further minimize oil transfer while maintaining or improving other properties, so as to approach optimum performance characteristics for a thermographic stencil sheet.

**SUMMARY OF THE INVENTION**

35 The present invention provides an improvement in a stencil sheet of the type disclosed in our application Ser. No. 136,373, which reduces oil transfer while maintaining and in many cases exceeding other prior performance characteristics.

40 In the invention, a thermoplastic polymeric hydrocarbon resin is incorporated in and forms a part of the heat-flowable coating composition of a stencil sheet of the type disclosed in application Ser. No. 136,373. As in such prior application, the resulting composition includes a thermoplastic film-forming material comprising a cellulose organic ester, and plasticizing material partially but incompletely compatible with the film-forming material. The hydrocarbon resin functions in the composition both as a plasticizer for the cellulose ester and as a film-forming 45 material, having, however, substantially lower film-forming strength than the cellulose ester. Therefore, the hydrocarbon resin is treated as a plasticizer while taking into account its film-forming properties in formulating a coating composition.

55 The stencil sheet of the present invention more particularly comprises an ink-pervious base sheet, and an ink-impervious coating thereon of a heat-flowable composition of a cellulose organic ester film-forming material, and plasticizing material partially but incompletely compatible with the film-forming material including a thermoplastic polymeric hydrocarbon resin having a total content of polymerized indenes and coumarones of at least about 30% by weight.

60 The invention also provides a method of making an imaged stencil sheet, wherein the new stencil sheet is employed in contact with a graphic original, image areas of the stencil sheet are subjected to heat generated in the original by infrared ray absorption to render the composition flowable in the stencil sheet image areas, and the composition is caused to flow from the image areas 65 and thereby form corresponding ink-transmitting image openings in the stencil sheet. Preferred embodiments of

the invention also, or alternatively, may be imaged mechanically.

A stencil sheet may be provided according to the present invention that reduces oil transfer to the lower level thus far achieved, the oil transfer being but a very small proportion of the transfer resulting from use of the preferred embodiments of application Ser. No. 136,373. Also, the invention in its preferred embodiments for thermographic imaging affords a marked increase in stencil sheet durability. At the same time, copy quality is maintained, and imaging speed is maintained and at times increased.

#### DESCRIPTION OF THE PREFERRED EMBODIMENTS

The stencil sheet of the invention includes a stencil base tissue sheet that may be formed of any suitable fiber, such as abaca fiber, abaca and wood fibers, kozo fiber, or polyester fiber, loosely arranged to provide a foraminous, highly permeable tissue. The tissue may weigh about 4½ to 12 pounds per 3,000 sq. ft. (24" by 36," 500 sheets). A heat-flowable coating composition, which is solid at ambient temperature, is applied to the base sheet at a rate of about 14 to 24 lbs. (dry basis), preferably about 21 lbs. per 3,000 sq. ft.

The heat-flowable coating composition preferably melts at a temperature of at least about 65° C., and it is further preferred that the coating composition melts in the range of about 65–180° C., more preferably, about 90–160° C. (A coating composition melting point as referred to herein is determined as the temperature at which the composition on a stencil sheet visibly melts or liquefies.)

The heat-flowable coating composition includes a cellulose organic ester film-forming material, which is capable of forming a continuous, cohesive, flexible, ink-impervious film. The cellulose ester melts or is plasticizable to melt in the range of about 65–180° C. Lower alkanoic acid esters of cellulose, especially 2- to 5-carbon acid esters are preferred. The preferred cellulose esters include cellulose acetate propionate, cellulose acetate butyrate, cellulose acetate valerate, cellulose propionate butyrate, cellulose propionate valerate, cellulose butyrate valerate, cellulose propionate, cellulose butyrate, and cellulose valerate. The cellulose ester preferably is employed in a proportion in the range of about 5–45% by volume (6–52% by weight), and more preferably about 14–30% by volume (16–36% by weight) of the coating composition, including the film-forming and plasticizing materials and exclusive of additives thereto. (It has been found in practice, consistent with theoretical considerations, that volume proportions are more significant than weight proportions when substitutions of one component for another are being considered. Accordingly, the proportions of the ingredients of the coating composition for the most part are set forth herein by volume.) The preferred cellulose esters have a minimum total butyryl and valeryl content of about 35% by weight and a maximum hydroxyl content of about 4.7% by weight. The most advantageous results are obtained by employing higher total butyryl and valeryl contents, at least about 44% by weight, and lower hydroxyl contents, about 2% by weight maximum. Optimally, the total butyryl and valeryl content is at least about 48% by weight, and the hydroxyl content is below about 0.7% by weight.

Cellulose acetate butyrate is the currently preferred cellulose ester, because it both furnishes a high quality product and is readily available in the market. Of the available grades of cellulose acetate butyrate, it is preferred to employ those having a butyryl content in the range of about 35% to 55% and preferably at least about 44–48%, as noted above. In the preferred grades, the average acetyl contents range from about 1.5% to 13.5%, and the hydroxyl contents range from as low as 0.1% to 4.7%, both on a weight basis. As noted above, the better products are obtained with the lower hydroxyl contents, below 2% and, preferably, below 0.7%. The preferred

grades have viscosities of about 0.07–6 seconds by A.S.T.M. Method D-1343-54T in Formula A, A.S.T.M. Method D-871-54T, and melting or softening points ranging from 125° C. to 185° C., preferably, at least about 150° C. (determined as the temperature at which a sample first appears wet.)

The cellulose ester film-forming material is combined in the coating composition with a plasticizing material partially but incompletely compatible therewith. Such plasticizing material is defined to mean material which when heated with the film-forming material in the proportions used forms a substantially homogenous single phase melt, and which when cooled from the melt to ambient or room temperature forms a two-phase mixture, at least one phase of the mixture incorporating substantial proportions of both the film-forming material and the plasticizing material.

The preferred embodiments of the coating composition of film-forming and plasticizing materials exhibit a transition between a single-phase mixture and a two-phase mixture at a temperature generally in the range of about 50–180° C. Such transition temperature is referred to herein as the compatibility temperature of the composition, and it is determined as the cloud point upon cooling the composition from a single phase melt. Thus, the first appearance of cloudiness signifies the transition from a single phase to two phases. In general, the transition is from a clear liquid to a cloudy liquid, but an obscuring material may be present without affecting performance.

Upon cooling below the compatibility temperature, the separation into two phases continues. The mixture remains fluid over a temperature range, and then the phase containing the major proportion of the film-forming material gradually hardens to a solid as the coating cools to room temperature. The remaining phase may solidify or remain liquid at room temperature. In the preferred embodiments, the remaining phase is a liquid at room temperature, forming a solid-liquid two-phase mixture thereat. The liquid phase may be trapped by the gel structure of the solid phase, or it may separate into a discrete liquid component.

As disclosed in application Ser. No. 136,373, the plasticizing material of the coating composition may constitute a single plasticizer, or may include a variety of plasticizers. Plasticizers are substantially non-volatile substances which serve to modify the physical properties of the cellulose ester film-forming material, including the melting or softening point, compatibility, and/or flow properties. They may be either liquid or solid at temperatures from ambient temperature up to close to imaging temperature, but at least must be fluid at imaging temperature in the complete plasticizing material component of the coating composition.

The plasticizers generally fall into three groups as regards compatibility with the film-forming material: Partially but incompletely compatible, incompatible, and compatible substances. Certain of the partially compatible plasticizers may be employed as sole plasticizers. Alternatively, two or more plasticizers having individual compatibilities ranging from complete compatibility to complete incompatibility may be employed, so long as the plasticizers together provide the proper balance of compatibility with the film-forming material. When a plurality of plasticizers is employed, it is highly preferable that they be compatible with each other at room temperature, forming a single phase mixture thereat, after heating together and cooling, if necessary for mixing.

The plasticizing material or complete plasticizer mix of the preferred coating composition is oleaginous or oily in nature, that is, it contains one or more oleaginous plasticizers. As disclosed in the above-identified earlier patent applications, numerous oleaginous plasticizers may be employed, such as mineral oil, castor oil, hexadecyl alcohol, polypropylene glycol monobutyl ether, polyoxethylene ethers of lanolin alcohols, pentaerythritol tetra-esters

of aliphatic acids having from 5 to 10 carbon atoms, trimethylol propane tri-esters of aliphatic acids having from 5 to 10 carbon atoms, rosin oil, polyoxethylene polyol fatty acid esters, and various other natural and synthetic oily materials. The hydrocarbon resin employed in the present invention may be oleaginous. Numerous other plasticizers, as disclosed in our aforesaid prior applications, also may be included in the coating composition.

A plasticizing material or complete plasticizer mix having certain additional physical properties has been found to be preferable. Thus, an amorphous plasticizing material having an optimum viscosity of about 40-110 Saybolt seconds at 99° C. is preferred for imaging purposes. It is preferred for minimizing migration and oiliness that the viscosity of any separable liquid phase remaining in a cooled melt of the coating composition be at least about 10 centipoises at 20° C. It is preferred for good aging properties that the plasticizing material have a maximum vapor pressure of about 0.1 mm. Hg at 30° C. and be substantially non-hygroscopic. It is preferred for resistance to emulsion type mimeograph inks that the plasticizing material have a maximum water solubility of about 1% at 30° C.

In the present invention, it is generally most advantageous and preferred, for reasons of performance, availability and economy, to employ a mineral oil together with the hydrocarbon resin in the plasticizing material or plasticizer mix having the foregoing character, although others of the above-described additional oleaginous plasticizers may be employed. Mineral oil and/or another of such oleaginous plasticizers preferably is present in a proportion in the range of about 10-70%, more preferably 15-65% by volume based on the total volume of the film-forming and plasticizing materials.

The preferred mineral oils, especially petroleum oils, have a viscosity below about 10,000 Saybolt seconds (SUS) at 38° C. and, more preferably, have a viscosity above about 30 Saybolt seconds at 38° C. Mineral oils having aniline points ranging from about 15° C. (mixed aniline point) to about 115° C. (straight aniline point) have proven to be satisfactory. In general, lower aniline point oils are preferred for use with lower compatibility cellulose esters, i.e., those esters having esterifying acyl groups of lower average molecular weight, and vice versa.

Aniline points as referred to herein and in the claims are determined in accordance with A.S.T.M. test D-1012-62, except where otherwise specified. Mixed aniline point is the minimum equilibrium solution temperature of a mixture of 2 volumes of aniline, 1 volume of sample, and 1 volume of n-heptane of specified purity. Straight aniline point is the minimum equilibrium solution temperature of a mixture of 1 volume of aniline and 1 volume of sample. Where the aniline point of a sample is too high or low for direct measurement, a material of known aniline point of opposite magnitude may be mixed with the sample for evaluation. The aniline point of the mixture is run, and the unknown aniline point is determined therefrom employing the formula:

$$A_u = \frac{A_m - A_k N_k}{N_u}$$

where  $A_u$  is the unknown aniline point,  $A_m$  is the aniline point of the mixture,  $A_k$  is the known aniline point, and  $N_k$  and  $N_u$  are the volumetric fractions of the known and unknown aniline point materials, respectively. Theoretical aniline points referred to hereinafter were determined in the foregoing manner. Similarly, aniline points of plasticizer mixtures may be calculated as the average of the aniline points of the individual plasticizers, as based on their relative proportions by volume. The aniline points set forth in the examples were determined in this manner.

A polymeric hydrocarbon resin is included in the plasticizing material in a preferred proportion of about 3-60%, more preferably 10-30% by volume, based on the total volume of film-forming and plasticizing materials including the resin. The preferred resins are synthetic thermoplastic resins derived from coal tar or petroleum, and more particularly, may be identified as polyindenes. They have a minimum of about 30%, preferably a minimum of 40% by weight of polymerized indenes and coumarones, including, particularly, polymers of indene, coumarone, and mono- and dimethyl derivatives thereof as found in the hydrocarbon resin product mixtures. The indenes and coumarones are referred to as bicyclic monomers.

Additionally preferred hydrocarbon resins are polymers having a monomer content that is substantially limited to indenes, coumarones, and styrenes, and may include aliphatic unsaturated monomers, particularly, cyclopentadienes. The styrenes as referred to herein, which are also termed vinyl aromatics, or monocyclic monomers, include styrene and derivatives thereof, such as the mono- and dimethyl ring- and side-chain substituted derivatives of styrene; ethyl styrene; divinyl benzene; and the like, as found in the hydrocarbon resin mixtures. Divinyl benzene while present in some resins is not a desirable monomer, and preferably, is limited to a maximum of about 3% by weight of the monomer content of a resin. The cyclopentadienes include, particularly, mono- and dicyclopentadiene, and mono- and dimethyl derivatives thereof, as also found in the hydrocarbon resin mixtures. The cyclopentadienes preferably are limited to a maximum of about 20%, more preferably, a maximum of about 10%, by weight of the monomer content of a resin.

It is further preferred that the hydrocarbon resin employed have a minimum of about 40% by weight of polymerized indenes and coumarones, and a minimum of about 80% by weight of polymerized aromatic "unsaturated" or aromatic "olefinic" monomers, including particularly, the indenes, coumarones, and styrenes, as described above. Any remaining monomer content of the resins may substantially constitute polymerized aliphatic (including cycloaliphatic) unsaturated or olefinic monomers, particularly, the cyclopentadienes as described above. Still further, it is preferred that the monomer content of the resin include at least about 80% of polymerized indenes and coumarones, the balance being substantially (one or more) polymerized styrenes. The latter resins are identified as coumarone-indene resins, commonly produced from the crude heavy solvent naphtha fraction of coal tar light oil, and also from certain carbureted water-gas oils.

The hydrocarbon resins useful in the invention may be liquid or solid at ambient temperatures, having softening points (Ring and Ball, A.S.T.M. E-28-42T) preferably in the range of about 5-175° C. The preferred resins of greater durability are solids at ambient temperatures and have softening points above about 50° C., more preferably, above about 90° C.

Useful hydrocarbon resins have a specific gravity (25° C., A.S.T.M. D-71) in the range of about 0.969-1.15, preferably about 1.016-1.145, and more preferably, about 1.132-1.145. The useful hydrocarbon resins have a refractive index ( $n_d^{25}$ ) in the range of about 1.53-1.65, preferably about 1.56-1.64, and more preferably about 1.62-1.64. Useful resins in general appear to have iodine numbers (Wijs, A.S.T.M. D-1959) less than about 100, a viscosity (Brookfield) of 1 poise at about 70-270° C., and a viscosity of 10 poises at about 40-220° C. It is preferred that the color be a maximum of about Gardner 14 (Neville 5), more preferably, Gardner 9 (Neville 2).

The preferred coal tar resins are produced by polymerization of monomers from crude heavy solvent naphthas, preferably boiling in the range of about 150-200° C. The principal monomers present are indene, methyl indenes,

coumarone, styrene, vinyl toluenes, and alpha-methyl styrene. The resins may be produced by polymerization of the monomers in the presence of a catalyst, including acid, clay and Friedel-Crafts catalysts. Typical processes are described in U.S. Pats. Nos. 1,990,215 and 2,565,222. Preferred coal tar resins include the coumarone-indene resins identified as Cumar resins (Neville Chemical Co.), including grades R-1, R-3, R-5, R-6, LX-509, R-7, R-9, R-10, R-11, R-12 and R-12A. Next in order of preference are Cumar resin grades R-13, R-14, R-15, R-16, R-17, RH-17, and R-19. Additional useful Cumar resin grades include R-21, R-27, R-28, R-29, P-10 and P-25.

The preferred petroleum hydrocarbon resins are produced by polymerization of by-product monomers obtained by high temperature, low pressure non-catalytic cracking of petroleum naphthas, natural gas, or gas-oil in the production of ethylene, propylene, butenes, butadiene, and/or isoprene. The monomers preferably boil within the range of about 100° C. to 300° C., contain as principal polymerizable components indene, methyl indenes, styrene and vinyl toluenes, and also may contain cyclopentadiene compounds. The resins may be produced by Friedel-Crafts polymerization of the monomers, as disclosed, in U.S. Pat. No. 3,422,053. A preferred resin produced in this manner is Neville LX-1517 (Neville Chemical Co.).

Additional useful hydrocarbon resins include Nevex 100 and Nevex 110 (Neville Chemical Co.), Resin EC-70 and Resin XL-30 (Velsicol Chemical Corp.), and Piccoumaron 410-HL and Piccoumaron 410-L (Pennsylvania Industrial Chemical Corp.). The useful hydrocarbon resins are low molecular weight polymers, preferably having average molecular weights less than about 2,000, more preferably, in the range of about 290-1600, and further preferably, in the range of about 400-1200 (as determined by vapor phase osmometer).

One or more additional plasticizers may be included in the coating composition if desired, where adjustment of one or more stencil properties is sought. Thus, for example, other plasticizing materials are disclosed in our prior applications Ser. No. 136,373 and Ser. No. 27,135, identified above. Also, as disclosed and claimed in co-pending application of the present inventors and Janis E. Wedyck, Ser. No. 253,394 filed May 15, 1972, enhanced durability may be achieved by the use of certain alkylene oxide reaction products of fatty acids and fatty alcohols, which are oleaginous plasticizers, as exemplified herein by the use of a preferred compound identified as Brij 92 (ICI America), described hereinafter. Further, it may be advantageous to incorporate with the coating composition finely divided silica gel, as disclosed and claimed in application Ser. No. 30,341, filed Apr. 20, 1970, by Leonard G. Larson and the present inventors, now U.S. Pat. No. 3,694,244. Applied with the composition of the present invention, the silica gel provides insurance against blocking, further minimizes oil transfer where less than optimum, and may provide an additional improvement in durability.

It appears preferable that the mixed aniline point of the complete plasticizing material or plasticizer mix in the composition be in the range of about 4-54° C. when employing cellulose acetate butyrate as the film-forming material, and more preferably, in the range of 21-54° C. with the preferred grades of cellulose acetate butyrate. In general, the compatibility of the cellulose ester film-former increases with the extent or proportion of acyl substitution, and the preferred aniline point of the plasticizing material increases with increased film-former compatibility, and vice versa. Thus, for example, the preferred plasticizer mixed aniline point when employing cellulose butyrate valerate, as exemplified hereinafter, is about 20° C. higher than for cellulose acetate butyrate. The hydrocarbon resin employed in the invention preferably has a mixed aniline point in the range of about 30-65° C. more preferably 45-60° C. One or more other plasticizers is blended with the hydrocarbon resin to provide the desired aniline point for the complete plasticizing material.

The specific film-forming and plasticizing materials and proportions thereof are selected on the basis of the herein defined properties. The film-forming and plasticizing materials are soluble in a volatile solvent and are also selected and blended in proportions so as to form a substantially homogeneous continuous imperforate coating when deposited from a solution thereof, the coating then being provided on the base sheet by deposition of the composition thereon from such solution. Preferably also, the coating is substantially clear, exclusive of the effect of additives other than the active or basic film-forming and plasticizing materials, i.e., additives such as the silica gel, pigments, fillers, and materials incorporated for other purposes. Reference to clarity is also exclusive of the opacifying effects of materials having an inherent opacity, such as waxy materials, and of the presence of materials which are solid at room temperature and are incorporated above their solubility limits at room temperature. Film-forming and plasticizing materials also are selected and blended in proportions such as to form a stencil sheet coating melting in the range of about 65-180° C.

When the materials satisfy the basic or preferred conditions, the proportions of individual materials then may be adjusted within limits to achieve optimum properties.

The composition of film-forming and plasticizing materials preferably is completely soluble in a volatile solvent at a temperature of below about 60° C., more preferably, at room temperature. The preferred compositions are soluble in organic solvent mixtures of an aromatic hydrocarbon, and an aliphatic ester and/or aliphatic alcohol. The composition is deposited on the base sheet from a solution in such solvent by evaporation of the solvent. The stencil coating formed in this manner is a uniform gel. The gel structure is changed so that the stencil coating is irreversibly physically altered when it is heated to its melting point, and also, at times, when it is heated to the compatibility temperature of the coating composition although lower than such melting point. Accordingly, the coated stencil base sheet is dried at a temperature below the melting point and the compatibility temperature, preferably at least 5° C. below the lower of the two temperatures.

In producing a stencil having optimum properties according to the invention, the following general sequence of evaluations may be followed:

At a selected proportion of cellulose ester, a mixture of plasticizers of diverse aniline points is combined and their relative proportions adjusted to vary the aniline point of the plasticizer mix until an aniline point optimum for the desired results is ascertained. In general, higher aniline points lead to better copy quality, slower imaging speed, more oil transfer, lower durability, better sensitivity for typing, and less blocking, and vice versa for lower aniline points. The proportion of the cellulose ester then is adjusted for optimum properties. In general, increasing the ester proportion at the same aniline point lowers the copy quality, reduces the imaging speed, decreases the oil transfer, increases the durability, reduces the sensitivity to typing, and reduces the blocking, and vice versa for decreasing ester proportions. The adjustment of the plasticizers for optimum aniline point then may be repeated with the optimum cellulose ester proportion.

A hydrocarbon resin according to the present invention is then selected and evaluated at various proportions, employing the optimum proportion of cellulose ester and with the resulting plasticizer mix at the optimum aniline point. The aniline point and/or the cellulose ester proportion may be adjusted once more to obtain a better balance of properties with the hydrocarbon resin present, if necessary. If desired, other plasticizers then may be substituted for the plasticizer or plasticizers employed with the hydrocarbon resin and/or the proportion of hydrocarbon resin may be varied with the introduction or removal of

other plasticizers, for improving the product in one or more respects, or making the product more attractive commercially, more adaptable to existing equipment or available materials, and so forth. It is also found that variations in the product may be desirable for certain types of ultimate use and/or reproduction equipment.

The stencil sheet may be imaged in a conventional thermographic machine, such as a roller-type copier as represented by Weber Thermal Imager, and a belt-type copier such as a Thermo-Fax Model 45CG "Secretary" machine. A tungsten filament lamp or other suitable source of infrared radiation is employed for imaging. A printed original in contact with the stencil sheet is exposed to radiation substantially instantaneously, i.e., on the order of about 0.03 to 0.1 second, to generate a temperature rise in the image portions of the original from about ambient temperature to a temperature sufficient to produce an imaging temperature in the image portions of the stencil sheet in the range of about 65-180° C.

The coating composition in the stencil sheet is heated to its melting point and is reduced to a flowable condition substantially instantaneously, and a part thereof is absorbed by the absorbent sheet or into adjacent areas of the stencil sheet immediately thereafter, to leave ink-transmitting image openings in the stencil sheet. The openings are bridged by the fibers of the stencil base sheet, which is ink-pervious, and the base sheet fibers serve to retain letter centers and the like in place. It is also found that a part of the coating solidifies in the image openings, after melting, and the solidified material in the openings then is in discrete particles, permitting free flow of ink around them when the stencil is employed for mimeograph duplication. After the stencil sheet is imaged, it is separated from the original and the absorbent sheet for use as a duplicating master.

In the examples which follow, the coating compositions were formulated in a solvent mixture of (in parts by weight) 50 parts of toluene, 35.8 parts of ethyl acetate, 14.2 parts of ethyl alcohol (95% denatured, U.S. Government Formula C), except where another solvent mixture is indicated. The cellulose ester was dissolved first in the solvent mixture, followed by dissolving the Brij 92 when employed. The hydrocarbon resin and any other plasticizers, except for the mineral oil, were then dissolved. The mineral oil when employed was added last, with mixing. When a silica gel was incorporated, it was dispersed in a portion of the solvent mixture, added to the solution of film-forming and plasticizing materials, and mixed well. In this manner, the materials of each coating composition were incorporated in the solvent mixture at a concentration of about 30-35% by weight.

Stencil base tissue sheet material made of abaca fiber was coated and impregnated with a coating composition. The tissue weighed 6.7 lbs. per 3,000 sq. ft. The sheet material was coated with the composition by contacting its bottom surface with the surface of a quantity of coating composition in a dish, removing excess fluid by a doctor rod, and drying by hanging the sheets in the atmosphere at room temperature. The total coated weight of the resulting stencil sheet ranged from 26 to 30 lbs. per 3,000 sq. ft. The thickness of the resulting stencil sheet was about 2 1/4 mils.

In addition to the listed ingredients, each coating composition included 0.17 gram of dilauryl thiopropionate antioxidant per 100 grams of active materials.

Each stencil sheet was assembled with an absorbent sheet for thermal imaging tests, in which imaging speed and copy quality were rated. The absorbent sheet was 10 lb. per 2,880 sq. ft. tissue formed of mixed abaca and wood pulp fibers (Grade 55 tissue, Dexter Corporation). Oil smudging of the original image was determined on carbon ribbon copy typed on bond paper, and oil transfer was determined on offset printed stock. Blocking was determined by storing unassembled stencil sheets in contact with each other in foil, at room temperature. Block-

ing was also determined in most cases by evaluating pinholing upon exposure with a blank sheet of coated paper in a thermal copier. Durability was determined on a Weber Model 50 (Weber Marking Systems) label printer type of mimeograph stencil duplicating machine.

Illustrative materials which may be employed in the invention, and referred to herein, are described as follows:

#### Cellulose Esters

10 CAB 500-1 is cellulose acetate butyrate grade EAB 500-1 (Eastman Chemical Products) having an average butyryl content of 49.6%, an average acetyl content of 5.5%, a hydroxyl content of 0.1-0.7%, a viscosity of 0.8-1.2 seconds determined by the hereinabove-identified ASTM method, and a melting point range of about 165-175° C.

CAB 500-5 is cellulose acetate butyrate grade EAB 500-5 (Eastman Chemical Products) having an average butyryl content of 48%, an average acetyl content of 6%, a hydroxyl content of 0.6-1.1%, a viscosity of 4-6 seconds (ASTM), and a melting point range of about 165-175° C.

CAB 381-2 is cellulose acetate butyrate grade EAB 381-2 (Eastman Chemical Products) having an average butyryl content of 37%, an average acetyl content of 13.5%, an average hydroxyl content of 2%, a viscosity of 1-3.5 seconds (ASTM), and a melting point range of 171-184° C.

Half-Second Butyrate (Eastman Chemical Products) 30 has an average butyryl content of 37%, an average acetyl content of 13.5%, an average hydroxyl content of 2%, a viscosity of 0.3-0.5 second (ASTM), and a melting point range of 155-165° C.

Tenth-Second Butyrate (Eastman Chemical Products) 35 has an average butyryl content of 37%, an average acetyl content of 13.5%, an average hydroxyl content of 2%, a viscosity of 0.01-0.16 second (ASTM), and a melting point range of about 155-165° C.

CAB 451-1 is cellulose acetate butyrate grade EAB 451-1 (Eastman Chemical Products) having an average butyryl content of 44%, an average acetyl content of 8.5%, an average hydroxyl content of about 1.3%, a viscosity of 1-2 seconds (ASTM), and a melting point range of 150-155° C.

45 CBV is cellulose butyrate valerate (Eastman Chemical Products) having an average valeryl content of about 46%, an average butyryl content of about 6%, a viscosity of 0.9 second (ASTM), and a melting point of about 120° C.

#### Silica Gel

Sylloid 255 (Davison Division, W. R. Grace Company) is silica gel having an oil absorption of about 315 lbs./100 lbs., a particle size range of 0.8-12 microns (90%), and an average particle size of about 3-4 microns.

#### Plasticizing Material

Mobilsol L (Socony Mobil Oil Co.) is a refined naphthenic petroleum oil having a viscosity of 61 Saybolt seconds (SUS) at 38° C., a straight aniline point of 74° C., an API gravity of 25.7°, and a distillation range of 254-370° C. (100%).

Brij 92 (ICI America) is polyoxyethylene ether of oleyl alcohol (2 moles of ethylene oxide) having an HLB (Atlas Hydrophile-Lipophile Balance) of 4.9, an acid number of 1.0 max., and a hydroxyl number of 160-180. It has a typical viscosity of approximately 30 centipoises at 25° C. (ASTM No. D445-53T), and a theoretical mixed aniline point of -2.8° C.

Staybelite Ester 5 (Hercules, Inc.), is a glycerol ester of hydrogenated rosin purified by steam distillation, typically having a softening point (Hercules drop method) of 81° C., an acid number of 5, a specific gravity of 1.06 at 25° C., and a mixed aniline point of 24.4° C.

Benol (Witco Chemical Company) is a white mineral oil typically having a viscosity of 100 Saybolt seconds at 38° C., a theoretical aniline point of 182° C., an API gravity of 34°, a distillation range of from 658 to 822° F. (100%), an ASTM cloud point of -10° C., an ASTM pour point of -12° C., and a flash point of 199° C.

Conoco DBCL (Continental Oil Company) is dedecylbenzylchloride (94.5%) having a viscosity of 101 Saybolt seconds at 38° C. and a mixed aniline point of 18° C.

Texanol Isobutyrate (Eastman Chemical Co.) is 2,2,4-trimethyl pentanediol diisobutyrate having a viscosity of 9 centipoises at 25° C., and a mixed aniline point of 8° C.

Flexol Plasticizer PEP (Union Carbide and Carbon Corp.) is di (isodecyl) 4,5-epoxy tetrahydrophthalate having a viscosity of 184 centipoises at 20° C. and a mixed aniline point of 7° C.

Bis-alpha-methyl benzyl ether (Union Carbide and Carbon Corp.) has a viscosity of 16.7 centipoises at 20° C. and a mixed aniline point of 22° C.

Atmul 122 (ICI America) is a solid of melting point approx. 52° C., composed of mono- and diglycerides of edible fats or oils, and containing a minimum of 54% monoglyceride (alpha form), and having a theoretical mixed aniline point of -1° C.

Conoco Paraffins (Continental Oil Co.) are normal C<sub>14</sub> to C<sub>16</sub> paraffins, containing 97-8% by weight of n-paraffins and 2.2% by weight maximum aromatics. The composition has a specific gravity of 0.78 at 16° C., a melting point

The preferred resin grades R-1, R-3, R-5, R-6, LX-509, R-7, R-9, R-10, R-11, R-12 and R-12A typically have the following more specific monomer composition:

5

| Monomer              | Range of proportions, percent by weight | Average proportion by weight |
|----------------------|-----------------------------------------|------------------------------|
| Indene               | 79.8-90.2                               | 85.0                         |
| Methyl indenes       | 0-6.3                                   | 2.0                          |
| Coumarone            | 1.9-10.0                                | 5.1                          |
| Styrene              | 0                                       | 0                            |
| Vinyl toluenes       | 3.2-11.5                                | 7.7                          |
| Alpha-methyl styrene | 0-1.7                                   | 0.2                          |

20

The foregoing preferred resin grades R-1 through R-12A are designated collectively as Type I resins. Resin grades R-13, R-14, R-15, R-16, R-17, RH-17, and R-19 are designated as Type II resins. Resin grades R-21, R-27, R-28, R-29, P-10 and P-25 are designated as Type III resins. The resins of the several types typically have the following physical properties:

|                                          | Type I      | Type II     | Type III    |
|------------------------------------------|-------------|-------------|-------------|
| 1. Softening point, °C                   | 98-165      | 56-105      | 7-48        |
| 2. Specific gravity, 25° C               | 1.321-1.145 | 1.016-1.127 | 0.969-1.099 |
| 3. Iodine number                         | 51-65       | 48-76       | 46-84       |
| 4. Mixed aniline point, °C               | 46-56       | 32-62       | 33-64       |
| 5. Molecular weight                      | 540-1,150   | 400-800     | 290-530     |
| 6. Temperature at 1 poise viscosity, °C  | 186-267     | 127-216     | 71-138      |
| 7. Temperature at 10 poise viscosity, °C | 151-220     | 102-171     | 44-98       |
| 8. Refractive index, 25° C               | 1.622-1.634 | 1.561-1.631 | 1.533-1.611 |

of 8° C., a viscosity of 2.7 centistokes at 38° C., and a mixed aniline point of 82° C.

Individual Cumar resins employed in the examples herein exhibited the following physical properties:

|                                          | R-9   | RH-17  | R-19   | LX-50       |
|------------------------------------------|-------|--------|--------|-------------|
| 1. Softening point, °C                   | 111.5 | 71.5   | 56     | 160-165     |
| 2. Specific gravity, 25° C               | 1.141 | 1.123  | 1.016  | 1.134       |
| 3. Iodine number                         | 51.2  | 63.1   | 53.5   | 58          |
| 4. Mixed aniline point, °C               | 46.8  | 42.0   | 58     | 55.8        |
| 5. Molecular weight                      | 613   | 445    | 591    | 1,090-1,148 |
| 6. Temperature at 1 poise viscosity, °C  | 195   | -----  | -----  | 267         |
| 7. Temperature at 10 poise viscosity, °C | 159   | -----  | -----  | 220         |
| 8. Refractive index, 25° C               | 1.632 | 1.6241 | 1.5607 | 1.634       |

Terpex Rosin Oil (SCM Glidden-Durkee) is a terpenic hydrocarbon oil having a specific gravity of 0.945 at 15.5° C., a Gardner-Holdt viscosity of H-K at 25° C., and a mixed aniline point of 54° C.

#### Hydrocarbon Resins

Cumar coumarone-indene resins (Neville Chemical Co.) identified by grade designations R-1, R-3, R-5, R-6, LX-509, R-7, R-9, R-10, R-11, R-12, R-12A, R-13, R-14, R-15, R-16, R-17, RH-17, R-19, R-21, R-27, R-28, R-29, P-10 and P-25 typically have the following monomer composition:

| Monomer              | Range of proportions, % by weight |
|----------------------|-----------------------------------|
| Indene               | 41.7-90.2                         |
| Methyl Indenes       | 0-6.3                             |
| Coumarone            | 0-10.0                            |
| Styrene              | 0-14.8                            |
| Vinyl Toluenes       | 3.2-37.0                          |
| Alpha-Methyl Styrene | 0-6.5                             |

Methods of analysis for the above-numbered properties of the Cumar resins were as follows:

1. ASTM D-28
2. ASTM D-71 for solid resins; Pycnometer for low melt, ASTM D-70
3. Neville N 12.09-56T (Modified Wijs)
4. ASTM D-611 modified (5 g. resin, 5 ml. n-heptane, 10 ml. aniline)
5. Vapor phase osmometer, number average, Mechrolab Model 301A
6. and 7. Brookfield viscosimeter, Model LTV
8. Extrapolation of 70% by weight resin in toluene above 25° C. softening point; determined on 100% resin having a softening point of 25° C. or less

Neville LX-1517 (Neville Chemical Co.) is a petroleum hydrocarbon resin produced by polymerization of petroleum naphtha fractions boiling in the range of 100-

300° C. and having the following typical monomer composition and physical properties:

| Monomer                        | Proportion, percent by weight |
|--------------------------------|-------------------------------|
| Indene                         | 24                            |
| Methyl Indenes                 | 19                            |
| Styrene                        | 19                            |
| Vinyl Toluenes                 | 23                            |
| Alpha-Methyl Styrene           | 3                             |
| Divinyl Benzene                | 2-3                           |
| Other C <sub>2</sub> -Styrenes | 9-10                          |

#### Physical Properties

|                                             |       |
|---------------------------------------------|-------|
| 1. Softening Point, ° C.                    | 103   |
| 2. Specific Gravity, 25° C.                 | 1.062 |
| 3. Iodine Number                            | 19-27 |
| 4. Mixed Aniline Point, ° C.                | 39.9  |
| 5. Molecular Weight                         | 840   |
| 6. Temperature at 1 poise viscosity, ° C.   | 205   |
| 7. Temperature at 10 poises viscosity, ° C. | 161   |
| 8. Refractive Index, 25° C.                 | 1.593 |

Nevex 100 and 110 (Neville Chemical Co.) are predominantly aromatic hydrocarbon resins having the following typical physical properties:

|                                             |             |
|---------------------------------------------|-------------|
| 1. Softening Point, ° C.                    | 102-109     |
| 2. Specific Gravity, 25° C.                 | 1.112-1.116 |
| 3. Iodine Number                            | 54-60       |
| 4. Mixed Aniline Point, ° C.                | 44.1-45.2   |
| 5. Molecular Weight                         | 602-699     |
| 6. Temperature at 1 poise viscosity, ° C.   | 184-192     |
| 7. Temperature at 10 poises viscosity, ° C. | 147-154     |
| 8. Refractive Index, 25° C.                 | 1.621-1.622 |

Piccoumaron 410-HL (Pennsylvania Industrial Chemical Corp.) is a hydrocarbon resin copolymer of primarily indene and vinyl aromatics (primarily styrene), in a weight ratio of 2.2-2.3 parts of indene per part of vinyl aromatics, having a softening point of 110-115° C., a specific gravity of 1.10, a refractive index of 1.63-1.64, a theoretical mixed aniline point of 46° C., an iodine number of 36, and a viscosity (Brookfield) of 1 poise at 195-200° C. and 10 poises at 165-170° C.

Resin EC-70 (Velsicol Chemical Corp.) is a hydrocarbon resin copolymer of 60% indenes, 10% coumarones and 30% styrene (estimated proportions by weight), typically having a softening point (Ring and Ball) of 112-118° C., a specific gravity of 1.08-1.11 (16° C.), a theoretical mixed aniline point of 48° C., and an iodine number of 80 max.

Resin XL-30 (Velsicol Chemical Corp.) is a hydrocarbon resin copolymer including indene and styrene, typically having a softening point (Ring and Ball) of 102-107° C., a specific gravity of 1.04-1.07 (16° C.), a refractive index of 1.6, a theoretical mixed aniline point of 40° C., a saponification number of 0-2, and an acid number of 0-2.

The following examples illustrate stencil sheets having various coating compositions according to the invention. In the examples, the aniline points refer to measurements on the mixture of plasticizers, exclusive of the cellulose ester, silica gel, pigments, and solvents. The volumetric relationships are significant only for the film-forming and plasticizing materials, which constitute the herein-termed "active" materials, and are calculated only for such materials. It will be understood that the invention is not limited to the examples, which are merely illustrative, or to the materials, proportions, conditions and procedures set forth therein.

#### EXAMPLE 1

Three coating compositions identified as A, B, and C were deposited on stencil base tissue, providing a total coated weight of about 26 lbs. per 3,000 sq. ft. with compositions A and B, and 27.5 lbs. per 3,000 sq. ft. with composition C. Compositions A and B varied in the grade of cellulose acetate butyrate, and compositions A and C

differed in that the latter included silica gel. The compositions were as follows:

#### EXAMPLE 1

| Material:                              | Composition       |         |         |
|----------------------------------------|-------------------|---------|---------|
|                                        | A                 | B       | C       |
| CAB 500-1                              | 16.85             | 16.85   | 19.9    |
| CAB 500-5                              |                   | 20.00   | 20.00   |
| Cumar R-9                              | 20.00             | 41.70   | 22.4    |
| Mobilsol L                             | 41.70             | 41.70   | 38.1    |
| Brij 92                                | 21.45             | 21.45   | 19.6    |
| Syloid 255                             |                   |         | 14.0    |
|                                        | Temperature, ° C. |         |         |
| Mixed aniline point of plasticizer mix | 48                | 48      | 48      |
| Compatibility temperature              | 130               | 127-130 | 130     |
| Melting point of stencil coating       | 116-127           | 128-135 | 116-127 |

<sup>1</sup> Composition C only.

Under several types of test conditions, the thermal imaging speeds of the three stencils were rated generally good, and their copy quality ratings were generally good.

Composition A had an oil smudging rating of very good and an oil transfer rating of good. Composition B had oil smudging and oil transfer ratings of good. Composition C, containing silica gel, was improved over composition A, having the ratings excellent for oil smudging and very good for oil transfer. None of the stencils exhibited blocking, for excellent ratings in this respect.

The durability of each stencil was high. The stencils from compositions A and C had desirable sensitivity for typing stencils, whereas typing sensitivity of the stencil from composition B was low. The stencil from composition C had excellent aging properties, determined upon storage for six months at 49° C.

The Cumar R-9 hydrocarbon resin employed in this and succeeding examples, as a preferred resin, and having the composition and properties described hereinabove, was made by the PB-Sulfuric process essentially as described in U.S. Pat. No. 1,990,215, from feed crude heavy solvent naphtha having the following typical properties (ASTM D-850):

|                                 |       |
|---------------------------------|-------|
| Specific Gravity, 15.6/15.6° C. | 0.965 |
| Distillation, ° C.:             |       |
| First drop                      | 164   |
| 5%                              | 172   |
| 10%                             | 174   |
| 50%                             | 178   |
| 90%                             | 182   |
| 95%                             | 185   |
| Decomposition                   | 194   |

#### EXAMPLE 2

The following compositions A and B were compared when deposited on stencil base tissue at respective total coated weights of about 27 and 28 lbs. per 3,000 sq. ft.:

| Material:                              | Composition       |       |
|----------------------------------------|-------------------|-------|
|                                        | A                 | B     |
| CAB 500-1                              | 18.00             | 18.00 |
| Cumar R-10                             | 21.20             |       |
| Mobilsol L                             | 38.20             | 46.30 |
| Brij 92                                | 22.60             | 14.50 |
| Staybelite Ester 5                     |                   | 21.20 |
|                                        | Temperature, ° C. |       |
| Mixed aniline point of plasticizer mix | 45                | 48    |

The essential change in composition A from composition B was the replacement of the plasticizer Staybelite Ester No. 5 by the hydrocarbon resin plasticizer Cumar R-10 pursuant to the present invention. The imaging speed increased from generally fair with the stencil from composition B to from good to very good with the stencil from composition A. Copy quality was good in both cases.

For composition B, oil smudging was rated good and oil transfer fair. Oil smudging and oil transfer both were rated excellent employing composition A. Blocking was excellent and durability was high in both cases. Typing sensitivity was similar and acceptable for both compositions.

The titanium dioxide and chrome yellow pigments were included to render the image visible by contrast, which is desirable when imaging mechanically. Thermal imaging speed was rated fair, and the copy quality was rated god. Oil smudging was rated very good, and oil transfer was rated excellent. Blocking was rated excellent. The typing sensitivity was relatively high. Stencil durability was rated medium.

#### EXAMPLE 4

10 The following coating compositions when deposited on stencil base tissue to provide a total coated weight of 26½ to 28½ lbs. per 3,000 sq. ft. resulted in improved stencil sheets according to the invention:

| Material:                                     | Composition |       |       |       |       |       |       |
|-----------------------------------------------|-------------|-------|-------|-------|-------|-------|-------|
|                                               | A           | B     | C     | D     | E     | F     | G     |
| Proportion, percent by volume                 |             |       |       |       |       |       |       |
| Half-second butyrate or tenth-second butyrate | 18.00       |       |       |       |       |       |       |
| CAB 451-2                                     |             | 18.00 |       |       |       |       |       |
| CBV                                           |             |       | 18.00 |       |       |       |       |
| CAB 500-1                                     |             |       |       | 16.85 | 16.85 | 18.00 |       |
| Cumar R-9                                     | 20.00       | 20.00 | 20.00 | 20.00 |       |       |       |
| Cumar RH-17                                   |             |       |       |       | 20.00 |       |       |
| Neville LX 1517                               |             |       |       |       |       | 20.00 |       |
| Resin XL-30                                   |             |       |       |       |       |       | 20.00 |
| Mobilsol L                                    | 18.30       | 18.20 | 30.20 | 47.20 | 43.75 | 35.00 | 43.30 |
| Benol                                         |             |       |       |       | 14.80 |       |       |
| Brij 92                                       | 43.70       | 43.80 | 31.80 |       | 19.40 | 28.15 | 18.70 |
| Temperature, °C.                              |             |       |       |       |       |       |       |
| Mixed aniline point of plasticizer mix        | 27          | 27    | 38    | 74    | 48    | 38    | 48    |

\*Coating composition solvent; 80% toluene, 20% ethanol (95%), by weight.

#### EXAMPLE 3

40

The following coating composition was deposited on stencil base tissue to provide a total coated weight of about 30 lbs. per 3,000 sq. ft.:

| Material                                             | Volume percent                          | 40 |
|------------------------------------------------------|-----------------------------------------|----|
| CAB 500-1                                            | 16.0.                                   |    |
| Cumar R-9                                            | 4.0.                                    |    |
| Mobilsol L                                           | 38.9.                                   |    |
| Brij 92                                              | 37.8.                                   |    |
| Titanium Dioxide grind (70% by weight in Castor Oil) | 2.5.                                    |    |
| Chrome Yellow grind (65% by weight in Castor Oil)    | 0.8.                                    |    |
| Syloid 255                                           | 3 lbs./100 lbs. of remaining materials. | 55 |

45 Except for composition C, having very high durability with low sensitivity, the stencil sheets are suitable for imaging by typewriter as well as thermographically.

#### EXAMPLE 5

50 The following coating compositions when deposited on stencil base tissue to provide a total coated weight of 26½ to 28½ lbs. per 3,000 sq. ft. resulted in improved stencil sheets according to the invention, suitable for imaging both thermographically and by typewriter:

| Material:                              | Composition |       |       |       |       |       |       |
|----------------------------------------|-------------|-------|-------|-------|-------|-------|-------|
|                                        | A           | B     | C     | D     | E     | F     | G     |
| Proportion, percent by volume          |             |       |       |       |       |       |       |
| CAB 500-1                              | 16.85       | 18.00 | 15.70 | 16.85 | 16.85 | 18.00 | 18.00 |
| Cumar LX-509                           | 20.00       |       |       |       |       |       |       |
| Nevex 100                              |             | 20.00 |       |       |       |       |       |
| Piccomararon 410-HL                    |             |       | 20.00 |       |       |       |       |
| Cumar R-19                             |             |       |       | 20.00 |       |       |       |
| Cumar R-21                             |             |       |       |       | 20.00 |       |       |
| Cumar R-27                             |             |       |       |       |       | 20.00 |       |
| Cumar P-10                             |             |       |       |       |       |       | 20.00 |
| Mobilsol L                             | 37.60       | 43.40 | 42.30 | 21.70 | 20.40 | 34.70 | 25.60 |
| Brij 92                                | 19.70       | 18.60 | 22.00 | 41.45 | 42.75 | 27.30 | 36.40 |
| Temperature, °C.                       |             |       |       |       |       |       |       |
| Mixed aniline point of plasticizer mix | 48          | 48    | 48    | 31    | 31    | 37    | 31    |
| Compatibility temperature              | 127         |       |       |       |       |       |       |

## EXAMPLE 6

The following coating compositions when deposited on stencil base tissue to provide a total coated weight of 26 to 28 lbs. per 3,000 sq. ft. resulted in improved stencil sheets according to the invention:

| Material:                              | Composition |       |       |       |       |
|----------------------------------------|-------------|-------|-------|-------|-------|
|                                        | A           | B     | C     | D     | E     |
| Proportion, percent by volume          |             |       |       |       |       |
| CAB 500-1                              | 15.70       | 16.85 | 16.85 | 16.85 | 16.85 |
| Cumar R-9                              | 20.00       | 20.00 | 20.00 | 25.00 | 20.00 |
| Mobilisol L                            | 34.30       | 38.20 | 38.80 | 29.00 | 47.20 |
| Conoco DBCL                            | 30.00       |       |       |       |       |
| Texanol isobutyrate                    |             | 24.95 |       |       |       |
| Flexol plasticizer PEP                 |             | 24.35 |       |       |       |
| Bis-alpha-methyl benzyl ether          |             |       | 29.15 |       |       |
| Atmuls 122                             |             |       |       | 15.45 |       |
| Temperature, °C.                       |             |       |       |       |       |
| Mixed aniline point of plasticizer mix | 48          | 48    | 48    | 48    | 53    |

## EXAMPLE 7

The following coating compositions when deposited on stencil base tissue to provide a total coated weight of 26 to 28½ lbs. per 3,000 sq. ft. resulted in improved stencil sheets according to the invention:

| Material:                                | Composition |       |       |       |       |
|------------------------------------------|-------------|-------|-------|-------|-------|
|                                          | A           | B     | C     | D     | E     |
| Proportion, percent by volume            |             |       |       |       |       |
| CAB 500-1                                | 15.70       | 25.00 | 15.70 | 16.85 | 16.85 |
| Cumar R-9                                | 10.00       | 20.00 | 20.00 | 20.00 | 20.00 |
| Mobilisol L                              | 49.00       | 36.30 |       |       |       |
| Conoco paraffins                         |             | 38.30 |       |       |       |
| Terpex rosin oil                         |             |       | 56.60 |       |       |
| Brij 92                                  | 25.30       | 18.70 | 26.00 | 6.55  |       |
| Polyoxyethylene polyol fatty acid ester* |             |       | 63.15 |       |       |
| Temperature, °C.                         |             |       |       |       |       |
| Mixed aniline point of plasticizer mix   | 48          | 48    | 48    | 48    | 40    |
| Compatibility temperature                | 93          |       |       |       |       |

\* Polyoxyethylene (40) sorbitol septoate, having an HLB value of 9, an acid number of 8-12, an hydroxyl number of 22-38, a saponification number of 100-110, a typical viscosity of 175 centipoises at 25° C., and a theoretical mixed aniline point of 37° C.

We claim:

1. In a stencil sheet including an ink-pervious base sheet, and an ink-impervious coating thereon of a heat-flowable composition of thermoplastic film-forming material comprising a cellulose organic ester, and plasticizing material partially but incompletely compatible with said film-forming material, the improvement which comprises

a thermoplastic polymeric hydrocarbon resin included in said plasticizing material in a proportion of about 3-60% by volume based on the total volume of the film-forming and plasticizing materials, said resin having a total content of polymerized indenes and coumarones of at least about 30% by weight, a maximum content of polymerized divinyl benzene of about 3% by weight, and a maximum content of polymerized cyclopentadienes of about 20% by weight, and said resin having a mixed aniline point of about 30-65° C., a softening point of about 5-175° C., and Brookfield viscosities of 1 poise at about 70-270° C. and 10 poises at about 40-220° C.

2. A stencil sheet as defined in claim 1 wherein the monomer content of said resin is substantially limited to indenes, coumarones, styrenes, and aliphatic unsaturated monomers, and said resin has a total content of polymerized indenes and coumarones of at least about 40% by weight, and a total content of polymerized indenes, coumarones, and styrenes of at least about 80% by weight. 75

3. A stencil sheet as defined in claim 1 wherein said resin is a coal-tar coumarone-indene resin having a total content of polymerized indenes and coumarones of at least about 80% by weight and the balance substantially polymerized styrenes.

4. A stencil sheet as defined in claim 3 wherein the softening point of said resin is in the range of about 90-175° C.

5. A stencil sheet as defined in claim 1 wherein said cellulose ester is selected from the group consisting of cellulose acetate propionate, cellulose acetate butyrate, cellulose acetate valerate, cellulose propionate butyrate, cellulose propionate valerate, cellulose butyrate valerate, cellulose propionate, cellulose butyrate, and cellulose valerate.

6. A stencil sheet as defined in claim 1 wherein said plasticizing material also includes a mineral oil.

7. In a stencil including an ink-pervious base sheet, and an ink-impervious coating thereon of a heat-flowable composition of thermoplastic film-forming material comprising a cellulose organic ester, and plasticizing material partially but incompletely compatible with said film-forming material including a mineral oil, the improvement which comprises

a thermoplastic polymeric hydrocarbon resin included in said plasticizing material, said resin having a total content of polymerized indenes and coumarones of at least about 30% by weight, a maximum content of polymerized divinyl benzene of about 3% by weight, and a maximum content of polymerized cyclopentadienes of about 20% by weight, and said resin having a mixed aniline point of about 30-65° C., a softening point of about 5-175° C., and Brookfield viscosities of 1 poise at about 70-270° C. and 10 poises at about 40-220° C.,

the proportions of said materials being about 5-45% of said ester, about 3-60% of said resin, and about 10-70% of said mineral oil, in proportions by volume based on the total volume of the film-forming and plasticizing materials.

8. A stencil sheet as defined in claim 7 wherein said cellulose ester is cellulose acetate butyrate.

9. A stencil sheet which comprises an ink-pervious base sheet, and an ink-impervious coating thereon of a heat-flowable composition of

thermoplastic film-forming material comprising a cellulose ester selected from the group consisting of cellulose acetate propionate, cellulose acetate butyrate, cellulose acetate valerate, cellulose propionate butyrate, cellulose propionate valerate, cellulose butyrate valerate, cellulose propionate, cellulose butyrate, and cellulose valerate, and

plasticizing material partially but incompletely compatible with said film-forming material including a thermoplastic polymeric hydrocarbon resin having a total content of polymerized indenes and coumarones of at least about 30% by weight, a maximum content of polymerized divinyl benzene of about 3% by weight, and a maximum content of polymerized cyclopentadienes of about 20% by weight, and said resin having a mixed aniline point of about 30-65° C., a softening point of about 5-175° C., and Brookfield viscosities of 1 poise at about 70-270° C. and 10 poises at about 40-220° C.,

the proportions of said materials being about 5-45% of said ester and about 3-60% of said resin, in proportions by volume based on the total volume of the film-forming and plasticizing materials,

said composition forming a substantially homogeneous single phase melt, and when cooled from the melt having a cloud point in the range of about 50-180° C., and forming a two-phase mixture at room temperature, at least one phase of said mixture incorporating substantial proportions of both said film-forming material and said plasticizing material,

said composition being soluble in a volatile solvent and forming a substantially homogeneous continuous imperforate coating when deposited from a solution thereof, and said coating being provided on said base sheet by deposition of said composition thereon from a solvent solution of the composition and removal of solvent therefrom, the melting point of said coating being in the range of about 65-180° C., said coating further becoming flowable and irreversibly physically altered when heated to its melting point for forming ink permeable image areas in the cooled stencil sheet.

10. A stencil sheet as defined in claim 9 wherein said cellulose ester has a minimum total butyryl and valeryl content of about 35% by weight, and a maximum hydroxyl content of about 4.7% by weight.

11. A stencil sheet as defined in claim 10 wherein the monomer content of said resin is substantially limited to indenes, coumarones, styrenes, and aliphatic unsaturated monomers, and said resin has a total content of polymerized indenes and coumarones of at least about 40% by weight, and a total content of polymerized indenes, coumarones, and styrenes of at least about 80% by weight.

12. A stencil sheet as defined in claim 11 wherein said plasticizing material also includes a mineral oil in a proportion of about 10-70% by volume based on the total volume of the film-forming and plasticizing materials.

13. A stencil sheet which comprises an ink-pervious base sheet, and an ink-impervious coating thereon of a heat-flowable composition of

thermoplastic film-forming material comprising cellulose acetate butyrate having a minimum butyryl content of about 35% by weight and a maximum hydroxyl content of about 4.7% by weight, plasticizing material partially but incompletely compatible with said film-forming material including

(a) a thermoplastic coal-tar coumarone-indene resin having a total content of polymerized indenes and coumarones of at least about 80% by weight and the balance substantially polymerized styrenes, a maximum content of polymerized divinyl benzene of about 3% by weight, and a maximum content of polymerized cyclopentadienes of about 20% by weight, and said resin having a mixed aniline point of about 30-65° C., a softening point of about 90-175° C., and Brookfield viscosities of 1 poise at about 70-270° C. and 10 poises at about 40-220° C., and

(b) a mineral oil,

the proportions of said materials being about 5-45% of said cellulose acetate butyrate, about 3-60% of said resin, and about 10-70% of said mineral oil, in proportions by volume based on the total volume of the film-forming and plasticizing materials, said composition forming a substantially homogeneous single phase melt, and when cooled from the melt having a cloud point in the range of about 50-180° C., and forming a two-phase mixture at room tem-

perature, at least one phase of said mixture incorporating substantial proportions of both said film-forming material and said plasticizing material, said composition being soluble in a volatile solvent and forming a substantially homogeneous continuous imperforate coating when deposited from a solution thereof, and said coating being provided on said base sheet by deposition of said composition thereon from a solvent solution of the composition and removal of solvent therefrom, the melting point of said coating being in the range of about 65-180° C., said coating further becoming flowable and irreversibly physically altered when heated to its melting point for forming ink-permeable image areas in the cooled stencil sheet.

14. A stencil sheet as defined in claim 13 containing, in proportions by volume based on the total volume of the film-forming and plasticizing materials, about 14-30% of said cellulose acetate butyrate, about 10-30% of said resin, and about 15-65% of said mineral oil, said cellulose acetate butyrate having a minimum butyryl content of about 44% by weight and a maximum hydroxyl content of about 2% by weight.

15. In a method of making an imaged stencil sheet employing a stencil sheet which includes an ink-impervious layer of a heat-flowable composition, wherein image areas of the stencil sheet are subjected to heat generated in adjacent image areas of an original by infrared ray absorption to render the composition flowable in the stencil sheet image areas and the composition is caused to flow therefrom and thereby form corresponding ink-transmitting image openings in the stencil sheet, the improvement which comprises employing as said stencil sheet the stencil sheet of claim 1.

35 16. A stencil sheet as defined in claim 1 wherein said resin has a total content of polymerized coumarones of up to about 10% by weight.

40 17. A stencil sheet as defined in claim 14 wherein said resin has a total content of polymerized coumarones of up to about 10% by weight.

## References Cited

UNITED STATES PATENTS

- |    |           |         |                        |          |
|----|-----------|---------|------------------------|----------|
| 45 | 3,704,155 | 11/1972 | Anderson et al. -----  | 117-35.5 |
|    | 1,790,987 | 2/1931  | Horii -----            | 117-35.5 |
|    | 1,792,095 | 2/1931  | Horii -----            | 117-35.5 |
|    | 2,808,777 | 10/1957 | Roshkind -----         | 117-36.1 |
|    | 3,062,675 | 11/1962 | Shelffo -----          | 117-35.5 |
| 50 | 3,120,611 | 2/1964  | Lind -----             | 117-36.1 |
|    | 3,177,086 | 4/1965  | Newman et al. -----    | 117-36.1 |
|    | 3,250,637 | 5/1966  | Frasher et al. -----   | 117-35.5 |
|    | 3,368,989 | 2/1968  | Wissinger et al. ----- | 117-36.1 |
|    | 3,446,662 | 5/1969  | Newman -----           | 117-36.1 |

MURRAY KATZ, Primary Examiner

U.S. CL. X.R.

UNITED STATES PATENT OFFICE  
CERTIFICATE OF CORRECTION

Patent No. 3,824,116 Dated July 16, 1974

Inventor(s) Bror E. Anderson and Margery L. Schick

It is certified that error appears in the above-identified patent and that said Letters Patent are hereby corrected as shown below:

Column 3, line 27: Change "melts" to --melt--;  
8, 54: Change "cersa" to --versa--;  
10, 37: Change "0.01" to 0.07--;  
11, 7: Change "dedecyl" to --dodecyl--;  
12, third table therein: Change the heading  
"LX-50" to --LX-509--.

Signed and sealed this 4th day of February 1975.

(SEAL)

Attest:

McCOY M. GIBSON JR.  
Attesting Officer

C. MARSHALL DANN  
Commissioner of Patents